

## UNITED STATES PATENT OFFICE

FRANK WAVRA, OF WOODRIVER, ILLINOIS

## MEANS AND METHOD OF MAKING LEATHER

No Drawing.

Application filed November 3, 1930. Serial No. 493,227.

This invention relates to certain new and useful improvements in means and method of making leather, the peculiarities of which will be hereinafter fully described and 5 claimed.

The main objects of my invention are, first, to produce tight leather and/or plump solid leather; second, to provide means to attain said objects; third, to provide a method 10 of using said means to attain said objects; and fourth, to save the hair.

I have found by practical use of my process that I can effect a very material saving of time in the treatment of hides for producing 15 leather, and obtain a strong plump and very tight leather, and also save the hair. To do this I soak the hides, and green flesh and re-soak two hours in fresh water. Then I add 6% lime with 1 1/4% concentrated sodium sulphide crystals of 60% strength (or the equivalent) in water to make 15% strength 20 solution, in three treatments in the paddle wheel, using one-third of above mixture successively on the same hides two hours apart, 25 to loosen the hair in 18 hours without destroying it.

For example, to treat a batch of 5000 lbs. of hides in 1800 gallons of water, I take 6% of 30 5000 lbs. equals 300 lbs. of lime, and mix it in about 150 gallons of cold water.

Then I take 1 1/4% of 5000 lbs. equals about 62 1/2 lbs. of concentrated sodium sulphide crystals of 60% strength, and dissolve it in about 25 gallons of boiling hot water making 35 15% solution. I pour this into the lime mixture and allow it to cool.

Then I take one-third of above lime and sodium sulphide mixture and add it to the 1800 gallons of water on the 5000 lbs. of hides. 40 These are stirred by paddles or otherwise agitated for 15 or 20 minutes and then are let stand until the end of two hours.

Then add another one-third of said mixture, agitate and let stand until the end of 45 the second two hour period.

Then add the final third of the above mixture, and agitate as above.

Allow the batch to stand for six hours. Then agitate 15 or 20 minutes and let stand for eight hours, making eighteen hours 50 treatment to loosen the hair.

To illustrate, after soaking, green fleshing and resoaking for two hours in fresh water as above stated, begin the first two hour period at (say) 1 p. m. by adding the first third 55 of said lime and sodium sulphide mixture and agitate.

Two hours later, at 3 p. m., add the second third of the lime and sodium sulphide mixture, and agitate.

Two hours later, at 5 p. m., give the third treatment as before.

Wait six hours, until 11 p. m., then agitate 15 to 20 minutes, and let stand until 7 a. m.,— 65 making up the said 18 hours of treatment.

During this time the temperature of the batch should be kept at 75 degrees to 80 degrees Fah. to obtain the best results.

Any other suitable process to loosen the hair may be used, before subjecting the hides 70 to my deliming or alkalining process described later.

After the said 18 hours, take out the hides and unhair by the usual process of machine or hand operation.

After unhauling put the hides back into a deliming or alkalining solution consisting of substantially the following proportions of the ingredients named: 250% clear water, 2.7% sodium sulphide, 2.5% lime, 0.5% sodium hydroxide, 4.0% common salt.

The hides are left in this alkaline solution from four to six hours. After this period wash the hides for 20 minutes in clear water.

Then soak the hides over night or about 85 eight hours, in a 2% salt water solution.

Then bathe the hides at least half an hour with half of 1% (that is 0.5%) Orapon, (a mixture of ammoniac and hardwood sawdust) at about 90 degrees F., and neutralize or 90

pickle in a solution consisting of: 0.5% formic acid, 44.0% salt, 0.25% wheat flour. Keep the hides in this solution for about 1 hour.

5 Then tan preferably with sodium bichromate or tanolin (a composition of sodium bichromate, sulphuric acid and corn sugar) for upper leather, which gives very tight and plump leather. For sole leather, 10 tan with vegetable or extract tan, which gives very plump or solid leather.

15 My process eliminates four days' time out of six days' time required by the usual process, and makes very tight upper leather, and 20 also plump and solid sole leather.

I do not limit myself to the exact proportions of the above named ingredients in the 25 solutions described, but give them as substantially the preferred proportions of means for carrying out my method of treating hides for 30 producing leather of improved quality.

I claim:

1. In the herein described treatment of 25 hides for producing improved leather, the process of stirring into a batch of soaked hides a solution of substantially 6% lime and 1 1/4% concentrated sodium sulphide crystals of 30 60% strength, or equivalent in three installments of one-third each and two hours apart, 35 waiting six hours, agitating 20 minutes, letting stand eight hours, taking out and unhairing, soaking in an alkalining solution, washing, soaking eight hours in a salt solution, 40 bating, pickling, and then tanning, substantially as described.

2. A composition of matter for producing 45 improved leather, the herein described alkalining solution consisting of sodium sulphide, lime, sodium hydroxide and common salt, dissolved in water.

3. A composition of matter for producing 50 improved leather, the herein described alkalining solution consisting of 2.7% sodium sulphide, 2.5% lime, 0.5% sodium hydroxide and 4.0% common salt, dissolved in 250% clear water.

4. A composition of matter for producing 55 improved leather, an alkalining process comprising soaking the hides in a solution of sodium sulphide, lime, sodium hydroxide and common salt, dissolved in water.

5. In the treatment of hides for producing 60 improved leather, the herein described alkalining process comprising soaking the hides about one hour in a solution of substantially the following proportions: 2.7% sodium sulphide, 2.5% lime, 0.5% sodium hydroxide and 4.0% common salt, dissolved in 250% clear water, substantially as described.

6. In the treatment of hides for producing 65 improved leather, the herein described process comprising adding to the soaked hides a solution of lime and concentrated sodium sulphide, letting stand and agitating at intervals for 18 hours at 75-80° Fah. taking out

70 and unhairing, then alkalining four to six hours in a solution of substantially the following proportions: 2.7% sodium sulphide, 2.5% lime, 0.5% sodium hydroxide and 4.0% common salt, dissolved in 250% clear water, then 75 washing in clear water, then soaking in a salt water solution, bating, pickling, and then tanning, substantially as described.

75 In testimony whereof I have affixed my signature.

FRANK WAVRA.

80

85

90

95

100

105

110

115

120

125

130